# EUROPEAN PATENT SPECIFICATION

(11) **EP 1 235 716 B1**
(45) Date of publication and mention of the grant of the patent: **06.09.2006**
(21) Application number: 00973065.6
(22) Date of filing: 06.11.2000
(51) Int. Cl.: B65D 1/02

(54) **MULTI-TRIP POLYESTER CONTAINERS WITH OXYGEN SCAVENGING MATERIAL**
EIN SAUERSTOFFABSORBIERENDES MATERIAL ENTHALTENDER UND WIEDERVERWENDBARER BEHÄLTER AUS POLYESTER
RECIPIENTS REUTILISABLES EN POLYESTER COMPORTANT UNE SUBSTANCE DESOXYGENANTE

(30) Priority: 11.11.1999 GB 9926601
(43) Date of publication of application: 04.09.2002
(73) Proprietor: Constar International Inc., Philadelphia, PA 19154 (US)
(72) Inventor: SERRANO, Francisco, Kempsey, Worcester WR5 3NB (GB)
(74) Representative: W.P. Thompson & Co.
(86) International application number: PCT/GB2000/004253
(87) International publication number: WO 2001/034479

(56) References cited:
- WO-A-89/01012
- WO-A-98/12127
- WO-A-99/38914

## Description

This invention relates to polyester containers, and particularly multilayer containers such as bottles for oxygen sensitive products such as beers and fruit juices etc.

Oxygen scavenging materials are known, such as those described in WO89/01012, in which a transition metal promotes the oxidation of an oxidisable polymer.
WO89/01012 gives as an example polyamide materials being oxidised by means of cobalt Siccatol (TM Akzo Chemie). Multilayer structures are envisaged as potential embodiments. ,

More recently multilayer bottles have been manufactured and sold in the US by Continental PET Technologies Inc. for beer products. These bottles appear to be five layer structures, with layers 1, 3 and 5 being formed from PET, and layers 2 and 4 from a polyamide material known as MXD6 further containing between 300 and 500 ppm cobalt. These bottles may have been made in accordance with the disclosure of WO99/38914, filed by Continental PET Technologies Inc.

This document discloses bottles and preforms according to the preamble of claims 1 and 12.

Measurements of the bottles show that the approximate thickness of the layers of these bottles are as follows:

| | | |
|---|---|---|
| Layer 1 | PET | 0.1025mm |
| Layer 2 | MXD6 + CO | 0.00625mm |
| Layer 3 | PET | 0.10625mm |
| Layer 4 | MXD6 + CO | 0.00875mm |
| Layer 5 | PET | 0.07mm |

Thus the total thickness of the PET layers is 0.27875mm and the oxygen scavenging (MXD6 + CO) layers is 0.015mm. The publicity on recyclying of these bottles, produced by Continental PET Technologies Inc, makes it clear that these bottles are "single trip" bottles.

According to the invention there is provided a polyester bottle comprising a neck portion, a side-wall portion, a shoulder portion interconnecting the neck and side-wall portions, and a base portion, the bottle consisting of three or more polymeric layers, at least the inner and outermost layers being formed of polyester, and one or more intermediate layers comprising an oxygen scavenging material, the total thickness of the polyester layers in the side-wall portion being at least 0.4mm, and the total thickness of the one or more intermediate layers in the side-wall portion being at least 0.02mm, the thickness of the polyester and intermediate layers being so as to provide a multi-trip polyester bottle.

Preferably the total thickness of the one or more intermediate layers in the side-wall portion is at least 0.025mm, and the total thickness of the polyester layers in the side-wall portion is at least 0.5mm. Whilst refillable multi-trip bottles are known per-se (as exemplified by EP0247566B), none of the prior art on bottles with oxygen scavenging materials envisages anything other than single trip bottles. Applicants believe they are the first to appreciate that oxygen scavenging materials can be used to design a multi-trip bottle and to design the bottle accordingly.

The oxygen scavenging material conveniently comprises an oxidisable organic polymer and a transition metal in a positive oxidation state. The oxidisable organic polymer is conveniently a polyamide, preferably a polymer containing units of the formula -NH-CH₂-arylene-CH₂-NH-CO-alkylene-CO-. The polyester is preferably polyethylene terephthalate. Preferably the bottle has three polymeric layers, an outermost layer of polyester, an innermost layer of polyester, and an intermediate layer comprising an oxidisable organic polymer and a transition metal in a positive oxidation state. The total thickness of the one or more intermediate layers preferably comprises approximately 5% of the total thickness of the side-wall portion.

The invention further resides in a preform for a polyester container, the preform comprising a neck portion, a side-wall portion to be drawn, and a closed bottom portion, the preform including three or more polymeric layers, at least the inner and outermost layers being formed of polyester, and one or more intermediate layers comprising an oxygen scavenging material, the total thickness of the polyester layers in the side-wall portion being at least 5mm, and the total thickness of the one or more intermediate layers in the side-wall portion being at least 0.3mm, the preform being suitable for the manufacture of a multi-trip polyester container. The total thickness of the one or more intermediate layers in the side-wall portion of the preform is preferably at least 0.35mm, and the total thickness of the polyester layers in the side-wall portion is at least 6mm, preferably at least 7mm.

The oxygen scavenging material conveniently comprises an oxidisable organic polymer and a transition metal in a positive oxidation state. The oxidisable organic polymer is conveniently a polyamide preferably a polymer containing units of the formula -NH-CH₂-arylene-CH₂-NH-CO-alkylene-CO-. The polyester is preferably polyethylene terephthalate. The preform preferably comprises three polymeric layers, an outermost layer of polyester, an innermost layer of polyester and an intermediate layer comprising an oxidisable organic polymer and a transition metal in a positive oxidation state. The total thickness of the one or more intermediate layers of the preform preferably comprises approximately 5% of the total thickness of the side-wall portion.

In addition to polyamides, the oxidisable organic polymer may be selected from a variety of polymers. Examples include ethylenically unsaturated hydrocarbons (for example as described in EP0507207A), polyolefins such as polypropylene and low density, medium density and high density polyethylene (e.g EP0451762A), ethylene vinyl copolymers such as EVOH (e.g US5281360), amines (e.g EP0542512), ascorbic acid (e.g WO91/17044), olefin-diene copolymers (e.g EP0713899A), and aliphatic polyketones (e.g W09813266). As can be seen from the above, many examples of oxygen scavengers comprising metal promoted oxidisable polymers have previously been proposed, but all for single trip containers. Cobalt neodecanoate and cobalt octoate are now preferred cobalt salts for use in these oxygen scavenging compositions.

The invention further resides in a method of providing a multi-trip polyester container comprising the steps of:
i) providing a multi-layer preform comprising three or more polymeric layers, including at least one layer comprising an oxygen scavenging material,
ii) stretch blow moulding the preform to form a blow moulded container body, characterised in that the container is capable of at least five re-use cycles, each including subjecting the container to a hot caustic wash at a temperature of at least 60°C (140°F) followed by product filling and capping, the container exhibiting substantially no crack failure following the five re-use cycles and dimensional stability to the extent that the maximum volume deviation over the five re-use cycles is a maximum of 1.5%.
Refillable containers must be able to withstand these stringent requirements, unlike single trip bottles.

Although such containers are designed to withstand in excess of five trips, and in excess of 100 weeks, it may be necessary to provide some marker means to indicate when the oxygen scavenging properties are nearing exhaustion and the container should no longer be reused. This marker means may be a relatively simple mechanism such as a date or batch code added to the container, or alternatively a more sophisticated mechanism such as an indicator adapted to change its visible appearance following a predetermined a time period after manufacture, or once the bottle has been exposed to a predetermined quantity of oxygen. Conceivably the colour of a marker, or of a layer of the container, conceivably the oxygen scavenging layer, could change under one or both of these conditions.

Accordingly the polyester bottle can include marker means adapted to indicate when the predetermined period of oxygen scavenging is close to expiry. In this way bottles can be accepted or rejected for reuse based on their estimated future oxygen barrier performance, regardless of the number of trips they have made or the age of the bottles. This allows the maximum acceptable usage of each bottle, whilst ensuring that certain minimum oxygen barrier capabilities are always met.

The invention will now be further described, by way of example only, with reference to the accompanying drawings, in which
Fig.1 is a schematic sectional view of a polyester preform in accordance with the present invention, and
Fig.2 is a schematic sectional view of a polyester bottle made from the preform of Fig.1 and in accordance with the present invention.

Referring to Fig.1, a polyester preform is shown generally at 1 and comprises a neck portion 2, a shoulder portion 3, a side-wall portion 4 and a base portion 5. The preform is formed mostly of polyethylene terephthalate, but is manufactured on a co-injection moulding machine such that there is an intermediate layer 6 of barrier material within the preform. The layer 6 does not extend substantially into the neck portion 2, and is discontinuous in the base portion 5.

The intermediate layer 6 divides the side-wall portion 4 into three layers, an outermost layer 7 of PET, the intermediate layer 6, and an innermost layer 8 again of PET. (The innermost layer 8 is "innermost" in the sense that it is towards the inner wall of the preform, as opposed to being towards the middle of the wall.) The outermost layer 7 of PET has a thickness of approx. 3.325mm, as does the innermost layer 8. The intermediate layer 6 has a thickness of approx. 0.35mm, and is formed of MXD6 polyamide (as sold by Mitsubishi Gas Chemicals of Japan) to which has been added 200 ppm cobalt neodecanoate. The total thickness of the side-wall portion 4 is approx. 7mm.

The preform 1 is then transferred to a stretch blow moulding machine and formed into the bottle of Fig.2. The bottle is shown generally at 9 and comprises the neck portion 2 (which is substantially unchanged), a shoulder portion 3' formed from the shoulder portion 3 of the preform, a side-wall portion 4' formed from the side-wall portion 4 of the preform, and a base portion 5' formed from the base portion 5 of the preform 1.

In the side-wall 4' of the blown bottle 9, an outermost PET layer 7' has a thickness of 0.2375mm, as does an innermost layer 8', with an intermediate layer 6' having a thickness of 0.025mm. The total thickness of the side-wall portion 4' is 0.5mm. These thicknesses are considerably in excess of those found in prior art multilayer bottles including oxygen scavenging compositions.

The bottle 9 is capable of at least 5 trips, each trip consisting of filling and capping, sale of the filled bottle and return of the empty bottle, and a caustic hot wash conventional in the reuse of multi-trip bottles. The intermediate layer 6' scavenges oxygen such that the bottle 9 has excellent oxygen barrier properties for a period in excess of 100 weeks. A marker patch (not shown) is present, for example on the underside of the base 5', to indicate when the 100 week period has been exceeded. In this way bottles nearing the end of their useful life may be removed from the refilling stream before the oxygen barrier performance is seriously affected.

## Claims

1. A polyester bottle comprising a neck portion (2), a side-wall portion (4'), a shoulder portion (3') interconnecting the neck (2) and side-wall (4') portions, and a base portion (5'), the bottle consisting of 3 or more polymeric layers, at least the inner and outermost layers being formed of polyester, and one or more intermediate layers comprising an oxygen scavenging material
**characterised in that** the total thickness of the polyester layers in the side-wall portion is at least 0.4mm, the total thickness of the one or more intermediate layers in the side-wall portion being at least 0.02mm and the thickness of the polyester and intermediate layers being so as to provide a multi-trip polyester bottle.

2. A polyester bottle according to claim 1
**characterised in that** the total thickness of the one or more intermediate layers in the side-wall portion is at least 0.025mm.

3. A polyester bottle according to claim 1 or claim 2,
**characterised in that** the total thickness of the bottle in the side-wall portion is at least 0.5mm.

4. A polyester bottle according to claim 1 or claim 2,
**characterised in that** the total thickness of the polyester layers in the side-wall portion is at least 0.5mm

5. A polyester bottle according to any of claims 1 to 4, **characterised in that** the one or more intermediate layers comprise an oxidisable organic polymer and a transition metal in a positive oxidation state.

6. A polyester bottle according to claim 5,
**characterised in that** the oxidisable organic polymer is a polyamide.

7. A polyester bottle according to claim 6,
**characterised in that** the oxidisable organic polymer is a polymer containing units of the formula -NH-CH₂-arylene-CH₂-NH-CO-alkylene-CO-.

8. A polyester bottle according to any preceding claim,
**characterised in that** the polyester is polyethylene terephthalate.

9. A polyester bottle according to any preceding claim,
**characterised in that** there are three polymeric layers, an outermost layer of polyester, an innermost layer of polyester and an intermediate layer comprising an oxidisable organic polymer and a transition metal in a positive oxidation state.

10. A polyester bottle according to any preceding claim,
**characterised in that** the total thickness of the one or more intermediate layers comprises approx. 5% of the total thickness of the side-wall portion.

11. A polyester bottle according to any preceding claim, wherein the bottle will scavenge oxygen during a predetermined period of oxygen scavenging,
**characterised in that** the bottle includes marker means adapted to indicate when the predetermined period of oxygen scavenging is close to expiry.

12. A preform (1) for a polyester container, the preform (1) comprising a neck portion (2), a side-wall portion (4) to be drawn, and a closed bottom portion (5), the preform including three or more polymeric layers, at least the inner and outermost layers being formed of polyester, and one or more intermediate layers comprising an oxygen scavenging material,
**characterised in that** the total thickness of the polyester layers is at least 5mm, and the total thickness of the one or more intermediate layers in the side-wall portion (4) is at least 0.3mm, the preform being suitable for the manufacture of a multi-trip polyester container.

13. A preform (1) according to claim 12,
**characterised in that** the total thickness of the one or more intermediate layers in the side-wall portion is at least 0.35mm.

14. A preform (1) according to claim 12 or claim 13,
**characterised in that** the total thickness of the polyester layers in the side-wall portion is at least 6mm.

15. A preform (1) according to claim 14,
**characterised in that** the total thickness of the polyester layers in the side-wall portion is at least 7mm.

16. A preform (1) according to any of claims 12 to 15,
**characterised in that** the one or more intermediate layers comprise an oxidisable organic polymer and a transition metal in a positive oxidation state.

17. A preform (1) according to claim 16,
**characterised in that** the oxidisable organic polymer is a polyamide.

18. A preform (1) according to claim 17,
**characterised in that** the oxidisable organic polymer is a polymer containing units of the formula -NH-CH₂-arylene-CH₂-NH-CO-alkylene-CO-.

19. A preform (1) according to any of claims 12 - 18,
**characterised in that** the polyester is polyethylene terephthalate.

20. A preform (1) according to any of claims 12 - 19,
**characterised in that** there are three polymeric layers, an outermost layer of polyester, an innermost layer of polyester, and an intermediate layer comprising an oxidisable organic polymer and a transition metal in a positive oxidation state.

21. A preform (1) according to any of claims 12 - 20,
**characterised in that** the total thickness of the one or more intermediate layers comprises approx. 5% of the total thickness of the side-wall portion.

22. A method of providing a multi-trip polyester container comprising the steps of:
i) providing a multilayer preform comprising three or more polymeric layers, including at least one layer comprising an oxygen scavenging material,
ii) stretch blow moulding the preform to form a blow moulded container body,
**characterised in that** the container is capable of at least five re-use cycles each, including subjecting the container to a hot caustic wash at a temperature of at least 60°C (140°F) followed by product filling and capping, the container exhibiting substantially no crack failure following the five re-use cycles and dimensional stability to the extent that the maximum volume deviation over the 5 re-use cycles is a maximum of 1.5%.

23. A method according to claim 21,
**characterised in that** the oxygen scavenging material is an oxidisable organic polymer and a transition metal in a positive oxidation state.

24. A method according to claim 22
**characterised in that** the oxidisable organic polymer, the transition metal and the respective amounts thereof are selected such that the layer will scavenge oxygen during a period of oxygen scavenging, the arrangement being such that the wall of the container body has a permeance to oxygen of not more than 0.5cm³/ (m² atm day) and the period of oxygen scavenging is such that following said five uses of the container, the wall of the container body has a permeance to oxygen of still not more than 0.5cm³/(m² atm day) provided said five uses are completed within an overall total period of 100 weeks.

## Patentansprüche

1. Polyesterflasche, die Folgendes umfasst: einen Halsabschnitt (2), einen Seitenwandabschnitt (4'), einen Schulterabschnitt (3'), der den Hals- (2) und den Seitenwandabschnitt (4') miteinander verbindet, und einen Basisabschnitt (5'), wobei die Flasche aus 3 oder mehr polymeren Lagen, von denen wenigstens die innere und die äußerste Lage aus Polyester gebildet sind, und ein oder mehreren Zwischenlagen besteht, die ein Sauerstoffbindungsmaterial beinhalten,
**dadurch gekennzeichnet, dass** die Gesamtdicke der Polyesterlagen im Seitenwandabschnitt wenigstens 0,4 mm beträgt, die Gesamtdicke der ein oder mehreren Zwischenlagen im Seitenwandabschnitt wenigstens 0,02 mm beträgt und die Dicke der Polyester- und Zwischenlagen derart ist, dass eine Multitrip-Polyesterflasche entsteht.

2. Polyesterflasche nach Anspruch 1, **dadurch gekennzeichnet, dass** die Gesamtdicke der ein oder mehreren Zwischenlagen im Seitenwandabschnitt wenigstens 0,025 mm beträgt.

3. Polyesterflasche nach Anspruch 1 oder Anspruch 2, **dadurch gekennzeichnet, dass** die Gesamtdicke der Flasche im Seitenwandabschnitt wenigstens 0,5 mm beträgt.

4. Polyesterflasche nach Anspruch 1 oder Anspruch 2, **dadurch gekennzeichnet, dass** die Gesamtdicke der Polyesterlagen im Seitenwandabschnitt wenigstens 0,5 mm beträgt.

5. Polyesterflasche nach einem der Ansprüche 1 bis 4, **dadurch gekennzeichnet, dass** die ein oder mehreren Zwischenlagen ein oxidierbares organisches Polymer und ein Übergangsmetall in einem positiven Oxidationszustand umfassen.

6. Polyesterflasche nach Anspruch 5, **dadurch gekennzeichnet, dass** das oxidierbare organische Polymer ein Polyamid ist.

7. Polyesterflasche nach Anspruch 6, **dadurch gekennzeichnet, dass** das oxidierbare organische Polymer ein Polymer ist, das Einheiten der Formel -NH-CH₂-Arylen-CH₂₋NH-CO-Alkylen-CO- enthält.

8. Polyesterflasche nach einem der vorherigen Ansprüche, **dadurch gekennzeichnet, dass** der Polyester ein Polyethylenterephthalat ist.

9. Polyesterflasche nach einem der vorherigen Ansprüche, **dadurch gekennzeichnet, dass** es drei polymere Lagen, eine äußerste Lage aus Polyester, eine innerste Lage aus Polyester und eine Zwischenlage gibt, die ein oxidierbares organisches Polymer und ein Übergangsmetall in einem positiven Oxidationszustand umfasst.

10. Polyesterflasche nach einem der vorherigen Ansprüche, **dadurch gekennzeichnet, dass** die Gesamtdicke der ein oder mehreren Zwischenlagen ca. 5% der Gesamtdicke des Seitenwandabschnitts umfasst.

11. Polyesterflasche nach einem der vorherigen Ansprüche, wobei die Flasche während einer vorbestimmten Sauerstoffbindungsperiode Sauerstoff bindet, **dadurch gekennzeichnet, dass** die Flasche Markierungsmittel beinhaltet, die anzeigen, wenn die vorbestimmte Sauerstoffbindungsperiode kurz vor dem Ende ist.

12. Vorformling (1) für einen Polyesterbehälter, wobei der Vorformling (1) Folgendes umfasst: einen Halsabschnitt (2), einen zu ziehenden Seitenwandabschnitt (4) und einen geschlossenen Bodenabschnitt (5), wobei der Vorformling drei oder mehr polymere Lagen beinhaltet, wobei wenigstens die innere und die äußerste Lage aus Polyester gebildet sind, sowie eine oder mehrere Zwischenlagen, die ein Sauerstoffbindungsmaterial umfassen,
**dadurch gekennzeichnet, dass** die Gesamtdicke der Polyesterlagen wenigstens 5 mm beträgt und die Gesamtdicke der ein oder mehreren Zwischenlagen im Seitenwandabschnitt (4) wenigstens 0,3 mm beträgt, wobei der Vorformling für die Herstellung eines Multitrip-Polyesterbehälters geeignet ist.

13. Vorformling (1) nach Anspruch 12, **dadurch gekennzeichnet, dass** die Gesamtdicke der ein oder mehreren Zwischenlagen im Seitenwandabschnitt wenigstens 0,35 mm beträgt.

14. Vorformling (1) nach Anspruch 12 oder Anspruch 13, **dadurch gekennzeichnet, dass** die Gesamtdicke der Polyesterlagen im Seitenwandabschnitt wenigstens 6 mm beträgt.

15. Vorformling (1) nach Anspruch 14, **dadurch gekennzeichnet, dass** die Gesamtdicke der Polyesterlagen im Seitenwandabschnitt wenigstens 7 mm beträgt.

16. Vorformling (1) nach einem der Ansprüche 12 bis 15, **dadurch gekennzeichnet, dass** die ein oder mehreren Zwischenlagen ein oxidierbares organisches Polymer und ein Übergangsmetall in einem positiven Oxidationszustand umfassen.

17. Vorformling (1) nach Anspruch 16, **dadurch gekennzeichnet, dass** das oxidierbare organische Polymer ein Polyamid ist.

18. Vorformling (1) nach Anspruch 17, **dadurch gekennzeichnet, dass** das oxidierbare organische Polymer ein Polymer ist, das Einheiten der Formel -NH-CH₂-Arylen-CH₂₋NH-CO-Alkylen-CO- enthält.

19. Vorformling (1) nach einem der Ansprüche 12 - 18, **dadurch gekennzeichnet, dass** der Polyester ein Polyethylenterephthalat ist.

20. Vorformling (1) nach einem der Ansprüche 12 - 19, **dadurch gekennzeichnet, dass** es drei polymere Lagen gibt, eine äußerste Lage aus Polyester, eine innerste Lage aus Polyester und eine Zwischenlage, die ein oxidierbares organisches Polymer und ein Übergangsmetall in einem positiven Oxidationszustand umfasst.

21. Vorformling (1) nach einem der Ansprüche 12 - 20, **dadurch gekennzeichnet, dass** die Gesamtdicke der ein oder mehreren Zwischenlagen ca. 5% der Gesamtdicke des Seitenwandabschnitts umfasst.

22. Verfahren zum Bereitstellen eines Multitrip-Polyesterbehälters, das die folgenden Schritte umfasst:
i) Bereitstellen eines mehrlagigen Vorformlings, der drei oder mehr polymere Lagen umfasst, einschließlich wenigstens einer Lage, die ein Sauerstoffbindungsmaterial beinhaltet,
ii) Streckblasen des Vorformlings zum Bilden eines streckgeblasenen Behälterkörpers,
**dadurch gekennzeichnet, dass** der Behälter wenigstens fünf Wiederverwendungszyklen durchlaufen kann, die jeweils das Unterziehen des Behälters einer Alkaliheißwäsche bei einer Temperatur von wenigstens 60°C (140°F), gefolgt von Produktabfüllung und Verschließen beinhalten, wobei der Behälter nach den fünf Wiederverwendungszyklen im Wesentlichen keine Risse aufweist und in dem Ausmaß maßstabil ist, dass die maximale Volumenabweichung nach den fünf Wiederverwendungszyklen maximal 1,5% beträgt.

23. Verfahren nach Anspruch 21, **dadurch gekennzeichnet, dass** das Sauerstoffbindungsmaterial ein oxidierbares organisches Polymer und ein Übergangsmetall in einem positiven Oxidationszustand ist.

24. Verfahren nach Anspruch 22,
**dadurch gekennzeichnet, dass** das oxidierbare organische Polymer, das Übergangsmetall und deren jeweilige Mengen so gewählt sind, dass die Lage während einer Sauerstoffbindungsperiode Sauerstoff bindet, wobei die Anordnung derart ist, dass die Wand des Behälterkörpers eine Sauerstoffdurchlässigkeit von nicht mehr als 0,5 cm³/(m² atm pro Tag) hat und die Sauerstoffbindungsperiode derart ist, dass nach den genannten fünf Verwendungen des Behälters die Wand des Behälterkörpers eine Sauerstoffdurchlässigkeit von immer noch höchstens 0,5 cm³/(m² atm pro Tag) hat, vorausgesetzt, dass die fünf Verwendungen innerhalb einer Gesamtperiode von 100 Wochen stattfinden.

## Revendications

1. Bouteille en polyester comprenant une partie de goulot (2), une partie de paroi latérale (4'), une partie d'épaulement (3') interconnectant les parties de goulot (2) et de paroi latérale (4'), et une partie de base (5'), la bouteille consistant en 3 couches polymériques ou plus, au moins les couches interne et externe étant formées de polyester, et une ou plusieurs couches intermédiaires comprenant un matériau épurateur d'oxygène
**caractérisée en ce que** l'épaisseur totale des couches de polyester dans la partie de paroi latérale est au moins de 0,4 mm, l'épaisseur totale des une ou plusieurs couches intermédiaires dans la partie de paroi latérale étant au moins de 0,02 mm et l'épaisseur des couches de polyester et intermédiaires étant prévue pour fournir une bouteille de polyester consignée.

2. Bouteille en polyester selon la revendication 1, **caractérisée en ce que** l'épaisseur totale des une ou plusieurs couches intermédiaires dans la partie de paroi latérale est au moins de 0,025 mm.

3. Bouteille en polyester selon la revendication 1 ou la revendication 2, **caractérisée en ce que** l'épaisseur totale de la bouteille dans la partie de paroi latérale est au moins de 0,5 mm.

4. Bouteille en polyester selon la revendication 1 ou la revendication 2, **caractérisée en ce que** l'épaisseur totale des couches de polyester dans la partie de paroi latérale est au moins de 0,5 mm.

5. Bouteille en polyester selon l'une quelconque des revendications 1 à 4, **caractérisée en ce que** les une ou plusieurs couches intermédiaires comprennent un polymère organique oxydable et un métal de transition dans un état d'oxydation positif.

6. Bouteille en polyester selon la revendication 5, **caractérisée en ce que** le polymère organique oxydable est un polyamide.

7. Bouteille en polyester selon la revendication 6, **caractérisée en ce que** le polymère organique oxydable est un polymère contenant des unités de la formule -NH-CH₂-arylène-CH₂-NH-CO-alkylène-CO-.

8. Bouteille en polyester selon l'une quelconque des revendications précédentes, **caractérisée en ce que** le polyester est du téréphthalate de polyéthylène.

9. Bouteille en polyester selon l'une quelconque des revendications précédentes, **caractérisée en ce qu'**elle compte trois couches polymériques, une couche externe de polyester, une couche interne de polyester et une couche intermédiaire comprenant un polymère organique oxydable et un métal de transition dans un état d'oxydation positif.

10. Bouteille en polyester selon l'une quelconque des revendications précédentes, **caractérisée en ce que** l'épaisseur totale des une ou plusieurs couches intermédiaires compose approximativement 5% de l'épaisseur totale de la partie de paroi latérale.

11. Bouteille en polyester selon l'une quelconque des revendications précédentes, dans laquelle la bouteille épurera l'oxygène durant une période prédéterminée d'épuration d'oxygène, **caractérisée en ce que** la bouteille comporte des moyens de marquage adaptés pour indiquer quand la période prédéterminée d'épuration d'oxygène est proche d'arriver à terme.

12. Préforme (1) de récipient en polyester, la préforme (1) comprenant une partie de goulot (2), une partie de paroi latérale (4) destinée à être extrudée, et une partie de fond fermé (5), la préforme comprenant trois couches polymériques ou plus, au moins les couches interne et externe étant formées de polyester, et une ou plusieurs couches intermédiaires comprenant un matériau épurateur d'oxygène,
**caractérisée en ce que** l'épaisseur totale des couches de polyester est au moins de 5 mm, et l'épaisseur totale des une ou plusieurs couches intermédiaires dans la partie de paroi latérale (4) est au moins de 0,3 mm, la préforme convenant pour la fabrication d'un récipient en polyester consigné.

13. Préforme (1) selon la revendication 12, **caractérisée en ce que** l'épaisseur totale des une ou plusieurs couches intermédiaires dans la partie de paroi latérale est au moins de 0,35 mm.

14. Préforme (1) selon la revendication 12 ou 13, **caractérisée en ce que** l'épaisseur totale des couches de polyester dans la partie de paroi latérale est au moins de 6 mm.

15. Préforme (1) selon la revendication 14, **caractérisée en ce que** l'épaisseur totale des couches de polyester dans la partie de paroi latérale est au moins de 7 mm.

16. Préforme (1) selon l'une quelconque des revendications 12 à 15, **caractérisée en ce que** les une ou plusieurs couches intermédiaires comprennent un polymère organique oxydable et un métal de transition dans un état d'oxydation positif.

17. Préforme (1) selon la revendication 16, **caractérisée en ce que** le polymère organique oxydable est un polyamide.

18. Préforme (1) selon la revendication 17, **caractérisée en ce que** le polymère organique oxydable est un polymère contenant des unités de la formule -NH-CH₂-arylène-CH₂-NH-CO-alkylène-CO-.

19. Préforme (1) selon l'une quelconque des revendications 12 à 18, **caractérisée en ce que** le polyester du téréphtalate de polyéthylène.

20. Préforme (1) selon l'une quelconque des revendications 12 à 19, **caractérisée en ce qu'**elle compte trois couches polymériques, une couche externe de polyester, une couche interne de polyester et une couche intermédiaire comprenant un polymère organique oxydable et un métal de transition dans un état d'oxydation positif.

21. Préforme (1) selon l'une quelconque des revendications 12 à 20, **caractérisée en ce que** l'épaisseur totale des une ou plusieurs couches intermédiaires compose approximativement 5% de l'épaisseur totale de la partie de paroi latérale.

22. Procédé de fourniture d'un récipient en polyester consigné comprenant les étapes de :
i) fourniture d'une préforme multicouche comprenant trois couches polymériques ou plus, comportant au moins une couche comprenant un matériau épurateur d'oxygène,
ii) moulage par extrusion-soufflage de la préforme afin de former un corps de récipient moulé par soufflage,
**caractérisé en ce que** le récipient peut faire l'objet d'au moins cinq cycles de réutilisation, comportant chacun un lavage caustique à chaud du récipient à une température d'au moins 60°C (140°F), puis le remplissage du produit et le bouchage, le récipient ne présentant substantiellement aucun défaut de fissure après les cinq cycles de réutilisation et une stabilité dimensionnelle telle que l'écart de volume maximum durant les 5 cycles de réutilisation est un maximum de 1,5 %.

23. Procédé selon la revendication 21, **caractérisé en ce que** le matériau épurateur d'oxygène est un polymère organique oxydable et un métal de transition dans un état d'oxydation positif.

24. Procédé selon la revendication 22, **caractérisé en ce que** le polymère organique oxydable, le métal de transition et les quantités respectives de ceux-ci sont sélectionnés de telle sorte que la couche épure l'oxygène durant une période d'épuration d'oxygène, l'agencement étant tel que la paroi du corps du récipient a une perméance à l'oxygène ne dépassant pas 0,5 cm³/(m² atm jour) et la période d'épuration d'oxygène est telle qu'après lesdites cinq utilisations du récipient, la paroi du corps du récipient a une perméance à l'oxygène ne dépassant toujours pas 0,5 cm³/(m² atm jour) à condition que lesdites cinq utilisations aient lieu durant une période totale globale de 100 semaines.
